# EUROPEAN PATENT SPECIFICATION

(11) **EP 0 271 005 B1**
(45) Date of publication and mention of the grant of the patent: **19.07.1995**
(21) Application number: 87117905.7
(22) Date of filing: 03.12.1987
(51) Int. Cl.: G03C 7/26, G03C 7/34

(54) **Silver halide photographic light-sensitive material excellent in dye-image preservability**
Photographisches lichtempfindliches Silberhalogenidmaterial, das in der Farbstoffbildhaltbarkeit ausgezeichnet ist
Matériau photographique à l'halogénure d'argent sensible à la lumière excellent en ce qui concerne la préservabilité de l'image de colorant

(30) Priority: 06.12.1986 JP 291277/86; 29.01.1987 JP 20101/87
(43) Date of publication of application: 15.06.1988
(73) Proprietor: KONICA CORPORATION, Tokyo 160 (JP)
(72) Inventor: Sasaki, Masao, Odawara-shi Kanagawa-ken (JP); Onodera, Kaoru, Odawara-shi Kanagawa-ken (JP); Komorita, Kazuo, Odawara-shi Kanagawa-ken (JP); Nakatsugawa, Hiroshi, Odawara-shi Kanagawa-ken (JP)
(74) Representative: Henkel, Feiler, Hänzel & Partner

(56) References cited:
- EP-A- 0 213 700

## Description

### Field of the Invention

This invention relates to a silver halide photographic light-sensitive material excellent in preservability of dye-image formed thereon.

### Background of the Invention

Generally, a silver halide color photographic light-sensitive material is coated on the support thereof with three kinds of silver halide color photographic emulsion layers selectively sensitized so as to enable the emulsion layers to have the sensitivity to a blue-light, green-light and red-light, respectively.

It is well-known that dye-images are generally faded or discolored in various preservation conditions of the above-mentioned color photographic light-sensitive materials. For example, like the display of color prints in the show window of a photo studio, there is a fading-discoloration caused in the case of preserving it being exposed to light for a long time. this type of fading-discoloration is called a light fading-discoloration. On the other hand, like the preservation of color prints in an album, there is another fading-discoloration caused when they are preserved in the dark at relatively high temperature and humidity for a long time, although an exposure to light is relatively short. This type of fading-discoloration is called a dark fading-discoloration.

When regarding photographic products including color prints as recording materials, it is demanded to reduce the above-mentioned fading-discoloration to the utmost even in any preservation conditions, and such demand is getting incresed year by year. Especially in cyan-dye forming couplers, the improvements of heat and moisture resistance thereof, i.e., a dark fading-discoloration resistance, have recently become an essential subject to be achieved.

The conventionally known cyan-dye forming couplers include, for example, a 2,5-diacylaminophenol type cyan-dye forming coupler substituted with an acylamino group in the 2nd and 5th positions of the phenol group of the coupler. They are described in, for example, U.S. Patent No. 2,895,826 and Japanese Patent Publication Open to public Inspection (hereinafter called Japanese Patent O.P.I. Publication) Nos. 112038-1975, 109630-1978 and 163537-1980.

These 2,5-diacylaminophenol type cyan-dye forming couplers are popularly used, because cyan dye-images excellent in dark-fading and discoloration resistance may be obtained. However, they have a defect in general that both of the light-fading resistance of color dye-images and the yellow discoloration, hereinafter simply called a Y-stain, of unreacted cyan-dye forming couplers caused by light are seriously inferior to others. Together with the above-mentioned light-fading, a phenomenon that a low density area is discolored into pink is particularly seen, so that even a problem of amplifying the visual color-fading may be caused.

Accordingly, as to the means of improving the light-fading resistance of such a 2,5-diacylaminophenol type cyan-dye forming coupler, there are proposed, for example, to use a benzotriazole compound in combination, as described in Japanese Patent O.P.I. Publication No. 151149-1975. However, this particular compound is serious in crystallization property, so that it cannot practically be used.

It is also known that such a high boiling organic solvent as dibutyl phthalate which has so far been used is used by inceasing its content. When having used this solvent, there has caused such a problem that photographic characteristics including color tones and the like are affected and dark-fading resistance is deteriorated; light-fading resistance may have been improved a little though. In addition, there has had few effects of inhibiting Y-stains caused by light.

On the other hand, Japanese Patent O.P.I. Publication No. 173835-1982 proposes a method of improving color tones and dye fastness in such a manner that, a 2,5-diacylaminophenol cyan-dye forming coupler substituted with an ortho-sulfonamidophenylacylamino group in the 2nd position of the phenol group of the cyan-dye forming coupler, such cyan-dye forming coupler is dispersed by making use of a high boiling organic solvent having a specific dielectric constant. With respect to the method, it was confirmed that the light-fading resistance of a cyan dye-image was seriously spoiled.

Further, Japanese Patent O.P.I. Publication No. 222852-1985 proposes a method of using both liquid type and solid type UV absorbers, and U.S. Patent No. 4,587,346 proposes a method of using a liquid type UV absorbent and other methods.

However, these methods have almost no effect particularly on the discoloration in a lowe density area; but a certain degree of effect on light-fading resistance though.

It is the present state of things that any method of obtaining cyan dye-images excellent in resistance against both dark-fading and light-fading and also in discoloration resistance in low density areas has not been discovered, and the improvements thereof have, therefore, been desired.

EP-A-0 213 700 belongs to the state of the art by virtue of Article 54(3) EPC and describes photographic material with a solid UV absorbing agent in an interlayer beneath a cyan coupler-containing layer.

### Summary of the Invention

It is, therefore, an object of the invention to provide a silver halide photographic light-sensitive mterial improved in light-fading resistance of cyan dye-images and, particularly, in discoloration resistance in low density areas of the images.

Another object of the invention is to provide a silver halide photographic light-sensitive material which is excellent in dark-fading resistance and is improved in dark-fading resistance.

Other objects of the invention will become apparent from the descriptions below.

The above-mentioned objects of the invention can be achieved with
a silver halide photographic light-sensitive material comprising a support having thereon
a silver halide emulsion layer containing a yellow dye-forming coupler,
a first interlayer,
a silver halide emulsion layer containing a magneta dye-forming coupler,
a second interlayer,
a silver halide emulsion layer containing a cyan dye-forming coupler,
a third interlayer and
a protective layer in this order from the support side,
wherein the cyan coupler is represented by the following formula [I] or [II] and each of the second and third interlayer comprises a liquid UV absorbing agent in the form of an amorphous and fluid liquid having an almost constant volume at 25°C together with at least one high boiling organic solvent having a dielectric constant of not more than 6.0 at 30°C in the ratio by weight of from 0.65 to zero to said UV absorbing agent contained in said layers;
wherein R₁ is an alkyl group or an aryl group; R₂ is an alkyl group, a cycloalkyl group, an aryl group or a heterocyclic group; R₃ is a hydrogen atom, a halogen atom, an alkyl group or an alkoxy group, provided that R₃ and R₁ may be bonded together to complete a ring; and Z₁ is a hydrogen atom or a group capable of releasing upon reaction with the oxidized product of a color developing agent.
wherein R₄ is an alkyl group having 2 to 6 carbon atoms; R₅ is a ballast group; and Z₂ is a hydrogen atom or an atom or a group capable of releasing upon reaction with the oxidized product of a color developing agent.

### Detailed Description of the Invention

The cyan-dye forming couplers used in the invention will now be described below.

In the cyan-dye forming couplers represented by Formula [I], hereinafter called the cyan-dye forming coupler of the invention, the preferable alkyl groups represented by R₁ are those having one to 32 carbon atoms. They may also be either straight-chained or branch-chained and include those having substituents.

The preferable aryl groups represented by R₁ are a phenyl group including those having substituents.

The preferable alkyl groups represented by R₂ are those having one to 32 carbon atoms. They may also be either straight-chained or branch-chained and include also those having substituents.

The preferable cycloalkyl groups represented by R₂ are those having 3 to 12 carbon atoms and they include also those having substituents.

The preferable aryl groups represented by R₂ are a phenyl group and include also those having substituents.

The preferable heterocyclic groups represented by R₂ are those of 5- to 7-membered, which may be either substituted or condensed.

R₃ is a hydrogen atom, a halogen atom, an alkyl group or an alkoxy group. Among them, a hydrogen atom is preferable.

The preferable rings completed by R₁ and R₃ bonded together are those of 5- or 6-membered. The examples of the 5- or 6-membered rings include the following rings:
and the like rings.

In Formula [I], the groups represented by Z₁ each capable of releasing upon reaction with the oxidized product of a color developing agent include, for example, a halogen atom, an alkoxy group, an aryloxy group, a acyloxy group, a sulfonyloxy group, an acylamino group, a sulfonylamino group, an alkoxycarbonyloxy group, an aryloxycarbonyloxy group, an imido group and the like and, preferably, a halogen atom, an aryloxy group and an alkoxy group.

The particularly preferable cyan-dye forming couplers of the invention are those represented by the following formula [I-A].
wherein R_{A1} is a phenyl group substituted with at least one halogen atom and such phenyl groups may further have other substituent than halogen atoms; R_{A2} is synonymous with R₁ denoted in the above-given Formula [I]; and Z_{A1} is a halogen atom, an aryloxy group or an alkoxy group.

The typical examples of the cyan-dye forming couplers represented by the Formula [I] will be given below:

The above-given cyan-dye forming couplers include 2,5-diacylamino type cyan-dye forming couplers described in, for example, Japanese Patent Application No. 21853-1986, pp.26-35; Japanese Patent O.P.I. Publication No. 225155-1985, the lower left column of p.7 to the lower right column of p.10; Japanese Patent O.P.I. Publication No. 222853-1985, the upper left column of p.6 to the lower right column of p.8; and Japanese Patent O.P.I. Publication No. 185335-1984, the lower left column of p.6 to the upper right column of p.9. These couplers may be synthesized in the methods described in the above-given specification.

Next, the cyan-dye forming couplers represented by the Formula [II] will be described.

In the Formula [II], the alkyl groups represented by R₄ may be either straight-chained or branch-chained and include those having substituents.

The ballst groups represented by R₅ are an organic groups each having such a size and a shape as are capable of giving couplers a sufficient volume so as not to diffuse the couplers substantially from a coupler-containing layers to other layers. The preferable ballast groups are those represented by the following formula:
wherein R₆ is an alkyl group having one to 12 carbon atoms; and Ar is such an aryl group as a phenyl group, which include those having substituents.

The typical examples of the couplers represented by Formula [II] will be given below. It is, however, to be understood that the invention shall not be limited thereto.

The typical examples of the cyan-dye forming couplers represented by Formula [II] including the above-given typical examples thereof are described in Japanese Patent Examined Publication No. 11572-1974, Japanese Patent O.P.I. Publication Nos. 3142-1986, 9652-1986, 9653-1986, 39045-1986, 50136-1986, 99141-1986 and 105545-1986, and so forth.

The cyan-dye forming couplers represented by Formula [I] or [II] may be used with other cyan-dye forming couplers in combination, provided that it shall not be contrary to the objects of the invention.

The cyan-dye forming couplers relating to the invention may be used in an amount within the range of, usually, from about 0.05 to 2 mol and, preferably, from 0.1 to one mol per mol of silver halide used.

The cyan-dye forming couplers relating to the invention is contained in a red-sensitive silver halide emulsion layer between the second and third interlayer and may also be contained in either a non-light-sensitive layer or an emulsion layer sensitive to the primary color spectral regions other than red spectral region.

In the invention, a liquid UV absorbing agent, hereinafter called the liquid UV absorbing agent of the invention, is used at an ordinary temperature.

In the invention, the expression, "liquid at an ordinary temperature", means an amorphous and fluid liquid having an almost constant volume at 25°C, as defined in 'Encyclopedia Chemica', 1963, Kyoritsu Publishing Co. and so forth. There is no limitation to the melting points thereof, provided they have the above-mentioned properties.

The liquid UV absorbing agents of the invention may be either a single compound or a mixture. As for such mixtures, those comprising a group consisting of structural isomers may preferably be used. (Such structural isomers are described in U.S. Patent No. 4,587,346 and so forth.)

The liquid UV absorbing agents of the invention may have any type of structures, provided that the above-mentioned requirements can be satisfied. From the viewpoint of the light-fastness of such UV absorbing agents themselves, it is preferable to use a 2-(2′-hydroxyphenyl)benzotriazole type compound represented by the following formula [a].

In the above-given Formula [a], R₁₁, R₁₂ and R₁₃ each are a hydrogen atom, a halogen atom, an alkyl group, an aryl group, an alkoxy group, an aryloxy group, an alkenyl group, a nitro group or a hydroxyl group.

The halogen atoms represented by R₁₁, R₁₂ and R₁₃ include, for example, a fluorine atom, an chlorine atom, a bromine atom and so forth and, among them, a chlorine atom is particularly preferable.

The alkyl and alkoxy groups represented by R₁₁, R₁₂ and R₁₃ include, preferably, those having one to 30 carbon atoms. The alkenyl groups preferably include those having 2 to 30 carbon atoms and these groups may be either straight-chained or branch-chained.

In addition, these alkyl, alkenyl and alkoxy groups may further have substituents.

The typical examples of the alkyl, alkenyl and alkoxy groups include, for example, a methyl group,. an ethyl group, an isopropyl group, a t-butyl group, a sec-butyl group, an n-butyl group, an n-amyl group, a sec-amyl group, a t-amyl group, an octyl group, a nonyl group, a dodecyl group, an eicosyl group, an α,α-dimethylbenzyl group, an octyloxycarbonylethyl group, a methoxy group, an ethoxy group, an octyloxy group, an allyl group and so forth.

The particularly preferable aryl and aryloxy groups out of those represented by R₁₁, R₁₂ and R₁₃ include, for example, a phenyl group and phenyloxy group and which may be substituted. The typical examples of such substituents include a phenyl group, a 4-t-butylphenyl group, a 2,4-di-t-amylphenyl group and so forth.

Out of the groups represented by R₁₁ and R₁₂, a hydrogen atom, an alkyl group, an alkoxy group and an aryl group is preferable and, in particular, a hydrogen atom, an alkyl group and an alkoxy group are more preferable.

Out of the groups represented by R₁₃, a hydrogen atom, a halogen atom, an alkyl group and an alkoxy group are particularly preferable and a hydrogen atom, an alkyl group and an alkoxy group are further preferable from the viewpoint of light-fading resistance.

In order to become liquid at an ordinary temperature, it is preferable that at least one group out of the groups represented by R₁₁, R₁₂ and R₁₃ is an alkyl group and it is more preferable that at least two groups are alkyl groups.

The alkyl groups represented by R₁₁, R₁₂ and R₁₃ may be of any types. It is, however, preferable that at least one is a tertiary alkyl group or a secondary alkyl group and it is particularly preferable that the alkyl group represented by at least one of R₁₁ and R₁₂ is a tertiary or secondary alkyl group.

The typical examples of the liquid UV absorbing agents relating to the invention will be given below:

The liquid UV absorbing agents relating to the invention may be added in any amount. However, the amount thereof added is, for example, within the range of from 0.1 to 300% by weight to the binder content of the photographic component layers each containing the UV absorbing agent, preferably within the range of from one to 200% and, more preferably, within the range of from 5 to 100%. The amount of the UV absorbing agent coated is preferably from 0.01 to 100 mg/100 cm², further preferably from 0.1 to 50 mg/100 cm² and still further preferably from 0.5 to 30 mg/100 cm².

In the invention, the aforementioned cyan-dye forming couplers relating to the invention are contained in the silver halide emulsion layer between the second and third interlayer and the above-mentioned liquid UV absorbing agent relating to the invention is contained in each of the second and third interlayer.

When adding the liquid UV absorbing agent relating to the invention to each of the second and third intermediate layers adjacent to a cyan-dye forming coupler-containing silver halide emulsion layer, the liquid UV absorbing agent relating to the invention is finely dispersed in a hydrophlic binder such as an aqueous gelatin solution by making use of a surface active agent, or by making use of a low boiling solvent such as ethyl acetate or the like, if required.

If required, it is also allowed to jointly use such a high boiling solvent as phenol derivatives, phthalic acid esters, phosphoric acid esters, citric acid esters, benzoic acid esters, alkyl amides, fatty acid esters, trimesic acid esters and so forth.

In addition to the above, the liquid UV absorbing agent relating to the invention may also be used at an ordinary temperature in combination with a solid UV absorbing agent. Even in this case, the above-mentioned adding method can also be applied.

In the case that the UV absorbing agent of the invention which is in liquid state at an ordinary temperature is jointly used at an ordinary temperature with as solid UV absorbing agent, it is particularly preferable that at least one kind of the liquid UV absorbing agent is jointly used with at least two kinds of solid UV absorbing agents.

Such combination of the above-mentioned UV absorbing agents are effective in preventing or inhibiting the surfaces of processed light-sensitive materials from fogging or causing the so-called haze.

The UV absorbing agents in solid state at an ordinary temperature preferably include the compounds which have the same formula [a] as that of the liquid UV absorbing agents and become solid at 25°C.

Now, the typical examples of the UV absorbing agents which are in solid state at an ordinary temperature will be given as follows:

In the above-mentioned case, any mixture proportion of a liquid UV absorbing agent to solid UV absorbing agents may be applied. However, in an ordinary temperature condition, the amount by weight of such a liquid UV absorbing agent is preferably not less than 30%, more preferably from not less than 30% to not more than 99% and, particularly from not less than 30% to not more than 95% to the whole UV absorbing agent used.

The solid UV absorbing agent is comprised of the combination of not less than 2 kinds of solid UV absorbing agents as the components of the above-mentioned absorbing agent and the component solid UV absorbing agents each have the different structures. At least one of the component solid UV absorbing agents has not less than 8 carbon atoms in total in the groups represented by R₁ and R₂ denoted in Formula [a]. The total content of all the component solid UV absorbing agents each having not less than 8 carbon atoms in total in the groups represented by R₁ and R₂ should preferably be not less than 35% by weight, more preferably be from not less than 35% upto 100% and particularly be from not less than 50% upto 100%.

However, the solid UV absorbing agent should preferably be comprised of not less than 2 kinds of the component solid UV absorbing agents having the different structures from each other, when the whole content of the component solid UV absorbing agents having not less than 8 carbon atoms in total in the groups represented by R₁ and R₂ is 100%.

In at least one of the UV absorbing agents which are in liquid state at an ordinary temperature, the groups represented by R₁ and R₂ nenoted in the aforegiven Formula [a] preferably have a total carbon number of not less than 8 and, however, the upper limit of the carbon numbers is preferably about not more than 12; such a upper limit may be varied by the groups represented by R₁ and R₂ and, further, by R₃ though.

Any of a total amount of both solid and liquid UV absorbing agents may be added, however, it is allowed to add them in total amount within the range of from 0.1 to 300% by weight to the amount of binders to be added to the photographic component layers each containing the UV absorbing agents respectively, and preferably from 1 to 200% and particularly from 5 to 100%.

A total amount of the respective UV absorbing agents to be coated is preferably from 0.01 to 100 mg/dm², more preferably from 0.1 to 50 mg/dm² and particularly from 0.5 to 30 mg/dm².

In the case that a silver halide photographic light-sensitive material of the invention used is a multicolor light-sensitive material, the arrangement of the component layers is that a silver halide emulsion layer containing a yellow dye-forming coupler, a first interlayer, a silver halide emulsion layer containing a magenta dye-forming coupler, a second interlayer, a silver halide emulsion layer containing the cyan dye-forming coupler relating to the invention, a third interlayer and a protective layer are arranged over to a support in order from the support side.

In the case that a silver halide photographic light-sensitive material of the invention has the above-mentioned layer arrangement, one of the liquid UV absorbing agents of the invention is contained in both of the second and third interlayers.

Also, in the invention, the layers containing the liquid UV absorbing agents further contain a high boiling organic solvent having a dielectric constant of not higher than 6.0 at 30°C in an amount within the range of from 0 to 0.65 parts by weight per part of a total amount of the UV absorbing agents added and preferably from 0 to 0.30 parts.

The above-mentioned high boiling organic solvents relating to the invention may be any compound, if it has a dielectric constant of not higher than 6.0. The lower limit of the dielectric constant thereof shall not be specially limitative, however, it is preferably not lower than 1.9. For example, such compounds include esters such as a phthalic acid ester, a phosphoric acid ester and the like; organic acid amides; ketons; hydrocarbon compounds; and so forth, and more preferably the phthalic acid esters or the phosphoric acid esters; provided that they have a dielectric constant of not higher than 6.0.

The preferable high boiling organic solvents are those having a vapor pressure of not higher than 0.5 mmHg at 100°C. Such organic solvents may be a mixture of two or more of them, provided that the dielectric constant thereof is not higher than 6.0. Every dielectric constant mentioned in the invention expresses those shown at 30°C.

The above-mentioned phthalic acid esters are represented by the following formula [HA]:
wherein R_{H1} and R_{H2} are each an alkyl group, an alkenyl group or an aryl group, provided that a total number of the carbon atoms of the groups represented by R_{H1} and R_{H2} is from 9 to 32 and more preferably from 16 to 24.

The alkyl groups represented by R_{H1} and R_{H2} in Formula [HA] are those straight-chained or branched and the include, for example, a butyl, hexyl, octyl, nonyl, dodecyl, tetra-decyl, hexadecyl, heptadecyl, octadecyl and the like groups.

The aryl groups represented by R_{H1} and R_{H2} include, for example, a phenyl, naphthyl and the like groups and, in addition, an alkenyl, hecenyl, heptenyl, octadeenyl and the like groups.

These alkyl, alkenyl and aryl groups are also allowed to have a single or plural substituents.

In the above-given Formula, the groups represented by R_{H1} and R_{H2} are preferably alkyl groups including, for example, 2-ethylhexyl group, 3,5,5-tromethylhexyl group, n-octyl group, n-nonyl group and the like groups.

The above-mentioned phosphoric acid esters are represented by the following formula [HB]:
wherein R_{H3}, R_{H4} and R_{H5} are each an alkyl, alkenyl or aryl group, provided that a total number of the carbon atoms of the groups represented by R_{H3}, R_{H4} and R_{H5} is from 24 to 54.

The alkyl groups represented by R_{H3}, R_{H4} and R_{H5} may be those straight-chained or branched which include, for example, a butyl, pentyl, hexyl, octyl, nonyl, dodecyl, pentadecyl, hexadecyl, octadecyl, nonadecyl and the like groups.

These alkyl, alkenyl and aryl groups are allowed to have a single or plural substituents. They groups represented by R_{H3}, R_{H}₄ and R_{H5} are preferably alkyl groups which include, for example, a 2-ethylhexyl, n-octyl, 3,5,5-trimethylhexayl, n-nonyl, n-decyl, sec-decyl, sec-dodecyl, t-octyl and the like groups.

The typical examples of the organic solvents will be given below and it is, however, to be understood that the invention shall not be limited thereto.

Among the high boiling organic solvents having a dielectric constant of not higher than 6.0, which may be used in the invention, the preferable ones are those represented by the above-given Formulas [HA] and [HB] and the more preferable ones are phthalic acid ester type high boiling organic solvents having the above-given Formula [HA].

In the silver halide light-sensitive material of the invention, it is allowed to contain simultaneously both of a high boiling organic solvent having a dielectric constant exceeding 6.0 and another one having a dielectric constant of not higher than 6.0. The total content of the former to that of the latter is not more than 0.5 by weight, preferably not more than 0.25 and further preferably not more than 0.1.

The silver halide photographic light-sensitive materials of the invention which have the above-mentioned structure may be in the forms of, for example, a color negative or positive film, a color print paper and the like and, inter alia, the advantages of the invention can effectively be displayed especially when they are used as a color print paper for direct appreciation of color photographs.

The dye-image forming couplers used in the invention shall not specially limited, except the cyan-dye forming couplers relating to the invention, but various types of such couplers may be used. For example, the typical ones include the following compounds:

The yellow-dye image forming couplers include, for example, those of the acylacetamide type and the benzoylmethane type.

The magenta-dye image forming couplers include, for example, those of the 5-pyrazolone type, pyrazolotriazole type, pyrazolinobenzimidazole type, indazolone type and cyanoacetyl type.

The silver halides used in the silver halide photographic light-sensitive materials of the invention include, for example, anyone used in the popular silver halide emulsions, such as silver bromide, silver iodobromide, silver iodochloride, silver chlorobromide, silver chloride and so forth.

The silver halide emulsions used in the invention may be chemically sensitized in, for example, a sulfur sensititization, a selenium sensitization, a reduction sensitization, a noble-metal sensitization and the like.

The silver halide emulsions used in the invention may be optically sensitized to a desired spectral wavelength region by making use of the dyes which are well-known as spectral sensitizing dyes in photographic industry.

As for the binders (or protective colloids) used in the silver halide photographic light-sensitive materials of the invention, gelatins may advantageously be used. Besides the gelatins, hydrophilic colloids may also be used, for example, gelatin derivatives, graft-polymers of gelatin and other macromolecules, proteins, sugar derivative, cellulose derivatives, synthesized hydrophilic macromolecular substances such as mono- or co-polymers.

If required, the silver halide photographic light-sensitive materials of the invention may further be added with additives such as a hardener, a color contamination inhibitor, an image stabilizer, a plasticizer, a latex, a surface active agent, a matting agent, a sliding agent, an antistatic agent and so forth.

The silver halide photographic light-sensitive materials of the invention may be able to form photographic images when they are treated in any color development processes which are well-known in the art.

As described above, the silver halide photographic light-sensitive materials of the invention are those which improved the light color-fading property of cyan-dye images and particularly eliminated the discoloration caused in low density areas, so as to form cyan color images which are stable against light, heat and moisture even if they are stored for a long time; and to reduce the possibility of changing cyan dyes into a leuco dyes during a development process.

### Examples

The invention will now be described in detail, with reference to the examples. It is, however, to be understood that the embodiments of the invention shall not be limited thereto.

### [Comparative Example-1]

There prepared a multilayered silver halide photographic light-sensitive material having the layer arrangement shown in Table-1, about which will be described in detail below.

AS-1, DS-1, Y-1, M-1 and UV-S1 used in the above compositions are the compounds having the following structures, respectively.

### Antistaining agent, AS-1

### Color-image stabilizer, DS-1

### Yellow coupler Y-1

### Magenta coupler M-1

### Solid UV absorbing agent UV-S1

These samples No. 1 through No. 23 were exposed to white light through an optical step wedge by making use of a photosensitometer (Model KS-7 manufactured by Konishiroku Photo Ind. Co., Ltd.) and were then processed in the following steps.

### Processing liquid composition

### (Color developer)

### (Bleach-fixer A)

With respect to the samples obtained from the above-mentioned process, the light color-fading, dark color-fading, yellow-staining and discoloring properties were tested in the following manner:

### [Light color-fading test]

By making use of an under-glass type outdoor exposure table, the samples were exposed to sun light for 5 days and for 15 days, respectively. The resulted light color-fading of each sample was expressed by the ratio of the residual color density of the respective cyan color images to the initial color density D=1.0 of the same images.

Residual ratio = (D/Do)x100, (in which D is a color density obtained after the color was faded.)

### [Dark color-fading test]

The samples were stored for 14 days in an atmosphere of a high temperature at 70°C and a high humidity at 80%RH, respectively. The resulted dark color-fading of each sample was expressed by the ratio of the residual color density of the respective cyan color images to the initial color density D=1.0 of the same images.

Residual ratio = (D/Do)x100, (in which D is a color density obtained after the color was faded.)

### [Yellow-staining test]

In both of the above-mentioned light and dark color fading tests, the degrees of the yellow stains (hereinafter sometimes simply called a YS) caused in each undeveloped color area were obtained in the following manner.

Yellow stain ΔD^{B} = D^{B} - Do^{B}, wherein
D^{B} = A blue-light density after stored, and
Do^{B} = A blue-light density before stored.

These samples were measured by making use of an optical densitometer (model PDA-65 manufactured by Konishiroku Photo Ind. Co., Ltd.).

### [Discoloration test]

In order to express the degrees of discoloration of cyan dye images, a 'P variation degree' is defined as follows.

When an initial cyan density (Dr) of 0.50 is disclored after test and both of a red-light density DR′ and green-light density DG are obtained after the discoloration. Thus, a discoloration degree P is expressed by a ratio (%) of the red-light density DR′ to the green-light density DG. Namely, a value of P (%) can be obtained by the following equation:$\text{P (%) = DG/DR′ x 100}$

Now, the dielectric constants of the high boiling organic solvents used in the example are shown below:

The results from the above-mentioned tests are collectively shown in Table-2 below.

It is found from the results shown in Table-2 that, as compared with Sample No. 1, Samples No. 2 through No. 5 and No. 23, that is, the samples containing a solid UV absorbing agent different from those of the invention and the samples containing a boiling organic solvent, an amount thereof added or a UV absorbent added to other layers each different from those of the invention, even if the liquid UV absorbing agents of the invention were added therein, such a sample has a problem that a pinkish discoloration is seriously caused; a light color-fading and light yellow-staining were somewhat improved though.

In contrast to the above-mentioned comparative samples, it is also found that Comparative Samples No. 6 through No. 22 obtained the excellent results satisfiable for every evaluation and displayed an excellent image preservability.

In addition to the above, Samples No. 6 through No. 13, No. 15 through No. 17, No. 19 through 21 and No. 22 each of which used the liquid UV absorbing agents not containing any halogen atom in R₁₃ denoted in the liquid UV absorbing agents represented by the aforegiven Formula [a] are more preferable from the viewpoint of pinkish discoloration prevention, and it is still further found that Samples No. 6, No. 8 through No. 16 and No. 20 through 22 each using a phthalic acid ester type high boiling organic solvents out of the high boiling organic solvents of the invention are also preferable from the viewpoint of dark yellow staining prevention.

The same effects were also found in Samples No. 19 and No. 20 which used the liquid UV absorbing agents of the invention to serve as a high organic solvent for the cyan-dye forming couplers of the invention.

### [Example-1]

Samples No. 31 through No. 44 were prepared in the same manner as in Comparative Example-1, except that the contents of UV absorbing agents, the layers containing the same and the kinds of cyan-dye forming couplers added to the 5th layers of each sample were changed as shown in Table-3, and the resulted samples were evaluated, respectively.

The UV absorbing agents, the high boiling organic solvents and the proportions by weight thereof were the same as in Comparative Example-1, and the details thereof are indicated by the respective sample numbers of Comparative Example-1.

The results obtained from the evaluation are shown in Table-3 below:

### Cyan-dye forming coupler *CC-1

### Solid UV absorbing agent *UV-2S

### Solid UV absorbing agent *UV-3S

From the results shown in Table-3, it is found that the effects of the invention can satisfactorily be displayed in Samples No. 34 and No. 36, No. 43 and No. 44, even in either cases where the constitutional requirements of the invention are applied to at least one or not less than two layers of the photographic component layers of the invention, or the different constitutional requirements are applied to the respective photographic component layers in Samples No. 41 and No. 42.

It is also found therefrom that there are particularly preferable results displayed, from the viewpoints of the prevention of both light fading and light yellow-staining, in Samples No. 36 through No. 42 and No. 44 each containing the constitutional requisites of the invention in the non-light-sensitive layer (that is the 6th layer) which was arranged to the opposite side of the cyan-dye forming coupler-containing silver halide emulsion layer of the invention, seeing from the support side.

### [Comparative Example-2]

The multilayered silver halide photographic light-sensitive material having the layer arrangement shown in Table-4 was prepared, of which will be described in detail below.

The resulted samples No. 51 through No. 66 were exposed to white light through an optical step wedge by making use of a sensitometer (Model KS-7 manufactured by Konishiroku Photo Ind. Co., Ltd.) and were then treated in the same process as in Comparative Example-1.

The treatments were made with bleach-fixer B having the same composition as in the aforementioned bleach-fixer A, except that 300 cc of the above-given developer were added to bleach-fixer A. After the treatments, the resulted samples were variously tested in the following manner.

### (1) Dark color-fading test

The samples were stored for 20 days in an atmosphere of a high temperature at 70°C and a high humidity at 80%RH, respectively. After then, each of the residual color-dye density (%) faded from the initial color density 1.0 of the dyes was measured.

### (2) Light color-fading test

The samples were irradiated with light by making use of a Xenon fade-o-meter (having 100,000 lux.) for 200 hours. After then, each of the residual color-dye density (%) faded from the initial color density 1.0 was measured.

### (3) Yellow-staining test

With respect to the samples irradiated with light for 200 hours in the above-mentioned test (2), the light yellow-stains (hereinafter sometimes simply called a light YS) caused in the undeveloped color areas were evaluated in the following manner.

Light YS: ΔDB = ΔDB - DoB, wherein
DB = A blue-light density after irradiation, and
DoB = A blue-light density after irradiation.

### (4) Cyan-color recurring test

Each of the maximum cyan-color density was obtained by processing with a color developer, bleach-fixer A and bleach-fixer B, respectively, was evaluated in the following manner.

Cyan-color recurring property (%) = DRB / DRA, wherein
- DRA:: A maximum cyan-color density obtained by processing with bleach-fixer A.
- DRB:: A maximum cyan-color density obtained by processing with bleach-fixer B.

The above-mentioned densities were measured by making use of an optiacal densitometer Model PDA-65 (manufactured by Konishiroku Photo Ind. Co., Ltd.)

The results obtained in the above-mentioned tests (1) through (4) are shown in Table-5. The dielectric constant of the high boiling organic solvent of the invention other than those given in Comparative Example-1 is as follow.

High boiling organic solvent No. H-7

The dielectric constant thereof is 4.4

The results are collectively shown in Table-5 below.

From the results shown in Table-5, it is found that Samples No. 52 through No. 54 each containing the cyan-dye forming coupler of the invention and the UV absorbing agent in combination have almost no effect on dark color-fading prevention and cyan-color recurring property; they are effective to some extent on the prevention of light color-fading and light yellow-staining though.

It is also found that Sample No. 55 containing the other cyan-dye forming coupler than that of the invention and the constitutional requisites for the invention in combination is seriously poor in the prevention of dark color-fading, in particular.

In contrast to the above, it is found that Samples No. 56 through No. 67 are endowed with excellent characteristics capable of answering to every evaluation so as to display the effects of the invention satisfactorily.

When the samples No. 56 through No. 67 were checked up in further detail, it is found that Samples No. 56 through No. 60 and No. 62 through No. 65 each not containing anu halogen atom in R₃ out of the liquid UV absorbing agents represented by Formula [a] are more preferable.

In addition to the above, it is found that Samples No. 56 through No. 63 using a phthalic acid ester type solvent out of the high boiling organic solvents or Sample No. 65 not using any high boiling organic solvent at all are particularly preferable from the viewpoint of light color-fading prevention.

### [Example-2]

Samples No. 71 through No. 83 were prepared in the same manner as in Comparative Example-2, except that the contents of both UV absorbing agents and high boiling organic solvents and the layers containing them were changed as shown in Table-6 and were then evaluated, respectively. The UV absorbing agents, high boiling organic solvents and the contents by weight thereof were the same as those in Comparative Example-2. The details thereof are indicated by the sample numbers of Comparative Example-2.

Besides the above, in the evaluation of color recurring property, bleach-fixer B used in Comparative Example-1 was replaced by the fatigued liquid having used in an automatic processor for processing color papers. The results obtained are shown in Table-6 below.

From the results shown in Table-6, it is found that these samples have displayed the effects of the invention satisfactorily even in either cases that the constitutional requisites of the invention were applied to not less than two photographic component layers or that the diffierent constitutional requisites were applied to the respective component layers.

It is also found therefrom that there are particularly preferable results displayed, from the viewpoints of the prevention of light color-fading, in Samples No. 76 through No. 81 and No. 83 each containing the constitutional requisites of the invention in the non-light-sensitive layer (that is the 6th layer) which was arranged to the opposite side of the cyan-dye forming coupler-containing layer, seeing from the support side.

On the other hand, it is found that Samples No. 77, No. 78 and No. 81 further improved in dark color-fading preventability and color-recurring property, so that the preferable results can be displayed.

### [Example-3]

In Samples No. 78 and No. 80 used in Example-4, cyan-dye forming coupler II-4 of the invention were replaced by II-8, II-9, II-12, II-14, II-16 and II-17, so that the samples for this example were prepared, respectively. The resulted samples were then evaluated in the same manner as in Example-2. It is found therefrom that the effects of the invention were displayed satisfactorily and the excellent results were obtained.

## Claims

1. A silver halide photographic light-sensitive material comprising a support having thereon
a silver halide emulsion layer containing a yellow dye-forming coupler,
a first interlayer,
a silver halide emulsion layer containing a magneta dye-forming coupler,
a second interlayer,
a silver halide emulsion layer containing a cyan dye-forming coupler,
a third interlayer and
a protective layer in this order from the support side,
wherein the cyan coupler is represented by the following formula [I] or [II] and each of the second and third interlayer comprises a liquid UV absorbing agent in the form of an amorphous and fluid.liquid having an almost constant volume at 25°C together with at least one high boiling organic solvent having a dielectric constant of not more than 6.0 at 30°C in the ratio by weight of from 0.65 to zero to said UV absorbing agent contained in said layers. wherein R₁ is an alkyl group or an aryl group; R₂ is an alkyl group, a cycloalkyl group, an aryl group or a heterocyclic group; R₃ is a hydrogen atom, a halogen atom, an alkyl group or an alkoxy group in which R₁ and R₃ may be bonded to each other to form a ring, and Z₁ is a hydrogen atom or a group capable of releasing upon reaction with the oxidized product of a color developing agent, wherein R₄ is an alkyl group containing two to six carbon atoms; R₅ is a ballast group and Z₂ is a hydrogen atom or a group capable of being releasing upon reaction with the oxidized product of a color developing agent.

2. The silver halide photographic light-sensitive material of claim 1, wherein said liquid UV absorbing agent is represented by the formula [a] wherein R₁₁, R₁₂ and R₁₃ are a hydrogen atom, a halogen atom, an alkyl group, an aryl group, an alkoxy group, an aryloxy group an alkenyl group, a nitro group or a hydroxy group, respectively.

3. The silver halide photographic light-sensitive material of claim 2, wherein R₁₃ is a hydrogen atom, an alkyl group or an alkoxy group.

4. The silver halide photographic light-sensitive material of claim 1, wherein an amount of said liquid UV absorbing agent is within the range of from 0.1% to 300%, preferably from 1% to 200%, particularly from 5% to 100% by weight to a binder contained in said layers containing said UV absorbing agent.

5. The silver halide photographic light-sensitive material of claim 1, wherein at least two solid UV absorbing agents of formula [a], respectively, wherein R₁₁, R₁₂ and R₁₃ are defined as in claim 2, which become solid state at 25°C, are contained in said layers together with said liquid UV absorbing agent.

6. The silver halide photographic light-sensitive material of claim 5, wherein the ratio by weight of the amount of said liquid UV absorbing agent to the total amount of said UV absorbing agents contained in said layers is not less than 30 %, preferably within the range from 30 % to 99 %, particularly within the range from 30 % to 95 %.

7. The silver halide photographic light-sensitive material of claim 5, wherein the total amount of said liquid UV absorbing agent and said solid UV absorbing agents is 0.1% to 300%, preferably 1 % to 200 %, particularly 5 % to 100 % by weight to a binder contained in said layers containing said UV absorbing agents.

8. The silver halide photographic light-sensitive material of claim 1, wherein an amount of said high boiling organic solvent is within the range of from 0.3 to zero parts per weight per part of the total amount of said liquid UV absorbing agent.

9. The silver halide photographic light-sensitive material of claim 1, wherein said high boiling organic solvent is not contained.

10. The silver halide photographic light-sensitive material of claim 1, wherein a dielectric constant of said high boiling organic solvent is within the range of from 1.9 to 6.0.

11. The silver halide photographic light-sensitive material of claim 1, wherein said high boiling organic solvent is a phthalate represented by the following formula [HA] : wherein R_{H1} and R_{H2} are each an alkyl group, an alkenyl group or an aryl group, provided that a total number of the carbon atoms of the groups represented by R_{H1} and R_{H2} is from 9 to 32.

12. The silver halide photographic light-sensitive material of claim 5, wherein an amount of said high boiling organic solvent is within the range of from 0.3 to zero parts by weight per part of the total amount of said UV absorbing agents.

13. The silver halide photographic light-sensitive material of claim 5, wherein said high boiling organic solvent is not contained.

14. The silver halide photographic light-sensitive material of claim 5, wherein a dielectric constant of said high boiling organic solvent is within the range of from 1.9 to 6.0.

15. The silver halide photographic light-sensitive material of claim 5, wherein said high boiling organic solvent is a phthalate represented by the formula [HA] wherein R_{H1} and R_{H2} are as defined in claim 11.

16. The silver halide photographic light-sensitive material of claim 1, wherein said high boiling organic solvent having a dielectric constant of not more than 6.0 at 30°C is the only high boiling solvent contained in said non-light-sensitive layers.

## Patentansprüche

1. Lichtempfindliches photographisches Silberhalogenid-Aufzeichnungsmaterial mit einem Schichtträger, auf dem sich - von der Schichtträgerseite her - in der angegebenen Reihenfolge
eine Silberhalogenidemulsionsschicht mit einem einen gelben Farbstoff bildenden Kuppler;
eine erste Zwischenschicht;
eine Silberhalogenidemulsionsschicht mit einem einen purpurroten Farbstoff bildenden Kuppler;
eine zweite Zwischenschicht;
eine Silberhalogenidemulsionsschicht mit einem einen blaugrünen Farbstoff bildenden Kuppler;
eine dritte Zwischenschicht und
eine Schutzschicht
befinden, wobei der Blaugrünkuppler durch folgende Formel [I] oder [II] wiedergegeben ist und sowohl die zweite als auch die dritte Zwischenschicht ein flüssiges UV-Absorptionsmittel in Form einer amorphen und fließfähigen Flüssigkeit eines nahezu konstanten Volumens bei 25°C zusammen mit mindestens einem hochsiedenden organischen Lösungsmittel einer Dielektrizitätskonstante von nicht mehr als 6,0 bei 30°C in einem Gewichtsanteil von 0,65 bis 0, bezogen auf das in diesen Schichten enthaltene UV-Absorptionsmittel, enthalten, worin bedeuten:
R₁ eine Alkylgruppe oder eine Arylgruppe;
R₂ eine Alkylgruppe, eine Cycloalkylgruppe, eine Arylgruppe oder eine heterocyclische Gruppe;
R₃ ein Wasserstoffatom, ein Halogenatom, eine Alkylgruppe oder eine Alkoxygruppe, wobei R₁ und R₃ miteinander unter Ringbildung verbunden sein können, und
Z₁ ein Wasserstoffatom oder eine bei der Reaktion mit dem Oxidationsprodukt einer Farbentwicklerverbindung freisetzbare Gruppe; worin bedeuten:
R₄ eine Alkylgruppe mit 2 bis 6 Kohlenstoffatomen; R₅ eine Ballastgruppe und
Z₂ ein Wasserstoffatom oder eine bei der Reaktion mit dem Oxidationsprodukt einer Farbentwicklerverbindung freisetzbare Gruppe.

2. Lichtempfindliches photographisches Silberhalogenid-Aufzeichnungsmaterial nach Anspruch 1, wobei das flüssige UV-Absorptionsmittel durch die Formel [a] worin R₁₁, R₁₂ und R₁₃ für ein Wasserstoffatom, ein Halogenatom, eine Alkylgruppe, eine Arylgruppe, eine Alkoxygruppe, eine Aryloxygruppe, eine Alkenylgruppe, eine Nitrogruppe oder eine Hydroxygruppe stehen, wiedergegeben ist.

3. Lichtempfindliches photographisches Silberhalogenid-Aufzeichnungsmaterial nach Anspruch 2, worin R₁₃ für ein Wasserstoffatom, eine Alkylgruppe oder eine Alkoxygruppe steht.

4. Lichtempfindliches photographisches Silberhalogenid-Aufzeichnungsmaterial nach Anspruch 1, wobei die Menge an dem flüssigen UV-Absorptionsmittel im Bereich von 0,1 - 300, zweckmäßigerweise 1 - 200, vorzugsweise 5 - 100 Gew.-%, bezogen auf ein in den das UV-Absorptionsmittel enthaltenden Schichten vorhandenes Bindemittel, liegt.

5. Lichtempfindliches photographisches Silberhalogenid-Aufzeichnungsmaterial nach Anspruch 1, wobei mindestens zwei feste UV-Absorptionsmittel der Formel [a] worin R₁₁, R₁₂ und R₁₃ die in Anspruch 2 angegebene Bedeutung besitzen, die bei 25°C in einen festen Zustand übergehen, zusammen mit dem flüssigen UV-Absorptionsmittel in den Schichten enthalten sind.

6. Lichtempfindliches photographisches Silberhalogenid-Aufzeichnungsmaterial nach Anspruch 5, wobei das Gewichtsverhältnis Menge an dem flüssigen UV-Absorptionsmittel/Gesamtmenge an den in den Schichten enthaltenen UV-Absorptionsmitteln nicht weniger als 30%, zweckmäßigerweise 30 - 99%, vorzugsweise 30 - 95% beträgt.

7. Lichtempfindliches photographisches Silberhalogenid-Aufzeichnungsmaterial nach Anspruch 5, wobei die Gesamtmenge an dem flüssigen UV-Absorptionsmittel und den festen UV-Absorptionsmitteln 0,1 - 300, zweckmäßigerweise 1 - 200, vorzugsweise 5 - 100 Gew.-%, bezogen auf ein in den die UV-Absorptionsmittel enthaltenden Schichten vorhandenes Bindemittel, liegt.

8. Lichtempfindliches photographisches Silberhalogenid-Aufzeichnungsmaterial nach Anspruch 1, wobei die Menge an dem hochsiedenden organischen Lösungsmittel im Bereich von 0,3 bis 0 Gew.-Teil pro Gew.-Teil der Gesamtmenge an dem flüssigen UV-Absorptionsmittel liegt.

9. Lichtempfindliches photographisches Silberhalogenid-Aufzeichnungsmaterial nach Anspruch 1, wobei das hochsiedende organische Lösungsmittel fehlt.

10. Lichtempfindliches photographisches Silberhalogenid-Aufzeichnungsmaterial nach Anspruch 1, wobei die Dielektrizitätskonstante des hochsiedenden organischen Lösungsmittels im Bereich von 1,9 - 6,0 liegt.

11. Lichtempfindliches photographisches Silberhalogenid-Aufzeichnungsmaterial nach Anspruch 1, wobei das hochsiedende organische Lösungsmittel aus einem Phthalat der folgenden Formel [HA] worin R_{H1} und R_{H2} jeweils für eine Alkylgruppe, eine Alkenylgruppe oder eine Arylgruppe stehen und die Gesamtzahl der Kohlenstoffatome der durch R_{H1} und R_{H2} dargestellten Gruppen 9 bis 32 beträgt, besteht.

12. Lichtempfindliches photographisches Silberhalogenid-Aufzeichnungsmaterial nach Anspruch 5, wobei die Menge an dem hochsiedenden organischen Lösungsmittel im Bereich von 0,3 - 0 Gew.-Teil pro Teil der Gesamtmenge an den UV-Absorptionsmitteln liegt.

13. Lichtempfindliches photographisches Silberhalogenid-Aufzeichnungsmaterial nach Anspruch 5, wobei das hochsiedende organische Lösungsmittel fehlt.

14. Lichtempfindliches photographisches Silberhalogenid-Aufzeichnungsmaterial nach Anspruch 5, wobei die Dielektrizitätskonstante des hochsiedenden organischen Lösungsmittels im Bereich von 1,9 bis 6,0 liegt.

15. Lichtempfindliches photographisches Silberhalogenid-Aufzeichnungsmaterial nach Anspruch 5, wobei das hochsiedende organische Lösungsmittel aus einem Phthalat der Formel [HA] worin R_{H1} und R_{H2} die in Anspruch 11 angegebene Bedeutung besitzen, besteht.

16. Lichtempfindliches photographisches Silberhalogenid-Aufzeichnungsmaterial nach Anspruch 1, wobei das hochsiedende organische Lösungsmittel einer Dielektrizitätskonstante von nicht mehr als 6,0 bei 30°C das einzige in den nicht lichtempfindlichen Schichten enthaltene, hochsiedende Lösungsmittel darstellt.

## Revendications

1. Un matériau photographique à l'halogénure d'argent sensible à la lumière, comportant un support qui porte
une couche d'émulsion d'halogénure d'argent contenant un coupleur de formation de colorant jaune,
une première intercouche,
une couche d'émulsion d'halogénure d'argent contenant un coupleur de formation de teinture magenta,
une deuxième intercouche,
une couche d'émulsion d'halogénure d'argent contenant un coupleur de formation de teinture cyan,
une troisième intercouche, et
une couche protectrice , dans cet ordre à partir de la face du support,
dans lequel le coupleur cyan est représenté par la formule suivante (I) ou (II) et chacune des deuxième et troisième intercouches comporte un agent liquide d'absorption des UV sous la forme d'un liquide amorphe et fluide présentant un volume presque constant à 25°C, conjointement avec au moins un solvant organique à point d'ébullition élevé présentant une constante diélectrique non supérieure à 6,0 à 30°C, dans le rapport pondéral de 0,65 à zéro par rapport audit agent d'absorption des UV contenu dans lesdites couches . dans laquelle R₁ est un groupe alkyle ou un groupe aryle ; R₂ est un groupe alkyle,un groupe cycloalkyle,un groupe aryle ou un groupe hétérocyclique ; R₃ est un atome d'hydrogène, un atome d'halogène, un groupe alkyle ou un groupe alkoxy, R₁ et R₃ pouvant être liés l'un à l'autre pour former un anneau, et Z₁ est un atome d'hydrogène ou un groupe capable d'être libéré lors de la réaction avec le produit oxydé d'un agent de développement couleur, dans laquelle R₄ est un groupe alkyle contenant deux à six atomes de carbone ; R₅ est une groupe ballast et Z₂ est un atome d'hydrogène ou un groupe capable d'être libéré lors de la réaction avec le produit oxydé d'un agent de développement couleur.

2. Le matériau photographique à l'halogénure d'argent sensible à la lumière de la revendication 1, dans lequel ledit agent liquide d'absorption des UV est représenté par la formule (a) dans laquelle R₁₁, R₁₂ et R₁₃ sont un atome d'hydrogène, un atome d'halogène, un groupe alkyle, un groupe aryle, un groupe alkoxy, un groupe aryloxy, un groupe alkényle, un groupe nitro ou un groupe hydroxy, respectivement.

3. Le matériau photographique à l'halogénure d'argent sensible à la lumière de la revendication 2, dans lequel R₁₃ est un atome d'hydrogène, un groupe alkyle ou un groupe alkoxy.

4. Le matériau photographique à l'halogénure d'argent sensible à la lumière de la revendication 1, dans lequel la quantité dudit agent liquide d'absorption des UV est située dans la plage de 0,1 % à 300 %, de préférence de 1 % à 200 %, en particulier de 5 % à 100 %, en poids d'un liant contenu dans lesdites couches contenant ledit agent d'absorption des UV.

5. Le matériau photographique à l'halogénure d'argent sensible à la lumière de la revendication 1, dans lequel au moins deux agents solides d'absorption des UV de formule (a), respectivement, dans laquelle R₁₁ , R₁₂ et R₁₃ sont définis dans la revendication 2, qui passent à l'état solide à 25°C, sont contenus dans lesdites couches conjointement avec ledit agent liquide d'absorption des UV.

6. Le matériau photographique à l'halogénure d'argent sensible à la lumière de la revendication 5, dans lequel le rapport pondéral de la quantité dudit agent liquide d'absorption des UV à la quantité totale desdits agents d'absorption des UV contenus dans lesdites couches n'est pas inférieur à 30%, de préférence dans la plage de 30 % à 99 %, en particulier dans la plage de 30 % à 95 %.

7. Le matériau photographique à l'halogénure d'argent sensible à la lumière de la revendication 5, dans lequel la quantité totale dudit agent liquide d'absorption des UV et desdits agents solides d'absorption des UV est, en poids, de 0,1 % à 300 %, de préférence de 1 % à 200 %, en particulier de 5 % à 100 %, par rapport à un liant contenu dans lesdites couches contenant lesdits agents d'absorption des UV.

8. Le matériau photographique à l'halogénure d'argent sensible à la lumière de la revendication 1, dans lequel la quantité dudit solvant organique à point d'ébullition élevé est dans la plage de 0,3 à 0 partie en poids par partie de la quantité totale dudit agent liquide d'absorption des UV.

9. Le matériau photographique à l'halogénure d'argent sensible à la lumière de la revendication 1, dans lequel ledit solvant organique à point d'ébullition élevé n'est pas présent.

10. Le matériau photographique à l'halogénure d'argent sensible à la lumière de la revendication 1, dans lequel la constante diélectrique dudit solvant organique à point d'ébullition élevé est dans la plage de 1,9 à 6,0.

11. Le matériau photographique à l'halogénure d'argent sensible à la lumière de la revendication 1, dans lequel ledit solvant organique à point d'ébullition élevé est un phtalate représenté par la formule suivante (HA) : dans laquelle R_{H1} et R_{H2} sont chacun un groupe alkyle, un groupe alkényle ou un groupe aryle, avec la condition que le nombre total des atomes de carbone des groupes représentés par R_{H1} et R_{H2} est de 9 à 32.

12. Le matériau photographique à l'halogénure d'argent sensible à la lumière de la revendication 5, dans lequel la quantité dudit solvant organique à point d'ébullition élevé est située dans la plage de 0,3 à zéro partie en poids par partie de la quantité totale desdits agents d'absorption des UV.

13. Le matériau photographique à l'halogénure d'argent sensible à la lumière de la revendication 5, dans lequel ledit solvant organique à point d'ébullition élevé n'est pas présent.

14. Le matériau photographique à l'halogénure d'argent sensible à la lumière de la revendication 5, dans lequel la constante électrique dudit solvant organique à point d'ébullition élevé est située dans la plage de 1,9 à 6,0.

15. Le matériau photographique à l'halogénure d'argent sensible à la lumière de la revendication 5, dans lequel ledit solvant organique à point d'ébullition élevé est un phtalate représenté par la formule (HA) dans laquelle R_{H1} et R_{H2} sont définis dans la revendication 11.

16. Le matériau photographique à l'halogénure d'argent sensible à la lumière de la revendication 1, dans lequel ledit solvant organique à point d'ébullition élevé présentant une constante diélectrique non supérieure à 6,0 à 30°C est le seul solvant à point d'ébullition élevé contenu dans lesdites couches non sensibles à la lumière.
